# EUROPEAN PATENT SPECIFICATION

(11) **EP 2 919 932 B1**
(45) Date of publication and mention of the grant of the patent: **23.03.2022**
(21) Application number: 13854766.6
(22) Date of filing: 19.11.2013
(51) Int. Cl.: B22D 25/06, B22D 21/00, B22C 9/22, B22D 2/00, B22D 19/14, C22C 1/10, C22C 32/00

(54) **METHOD OF PREPARING A CAST ALUMINIUM COMPOSITE MATERIAL**
VERFAHREN ZUR VORBEREITUNG EINES ALUMINIUM-GUSS-VERBUNDMATERIALS
PROCEDE DE PREPARATION D'UN MATERIAU COMPOSITE DE FONDERIE EN ALUMINIUM

(30) Priority: 19.11.2012 US 201261727949 P
(43) Date of publication of application: 23.09.2015
(73) Proprietor: Rio Tinto Alcan International Limited, Montréal, QC H3A 3G2 (CA)
(72) Inventor: LANGLAIS, Joseph, Jonquière, Québec G7X 4G5 (CA); ANDRADE, Neivi, Contrecoeur, Québec J0L 1C0 (CA); LAURIN, Jean-Alain, Jonquière (Québec) G7X 3P8 (CA)
(74) Representative: Germain Maureau
(86) International application number: PCT/CA2013/050881
(87) International publication number: WO 2014/075194

(56) References cited:
- CA-A1- 2 491 429
- CA-A1- 2 491 429
- US-A1- 2003 175 543
- US-A1- 2009 263 277
- US-A1- 2009 263 277
- US-B2- 7 562 692
- US-B2- 7 562 692
- LAI J ET AL: "Effect of Sc, Zr, and Ti on the interfacial reactions of the BC/Al system", JOURNAL OF MATERIALS SCIENCE, KLUWER ACADEMIC PUBLISHERS, BO, vol. 46, no. 2, 28 September 2010 (2010-09-28), pages 451-459, XP019854901, ISSN: 1573-4803, DOI: 10.1007/S10853-010-4914-5
- ZHANG Z ET AL: "Effect of titanium on microstructure and fluidity of Al-BC composites", JOURNAL OF MATERIALS SCIENCE, KLUWER ACADEMIC PUBLISHERS, BO, vol. 46, no. 9, 7 January 2011 (2011-01-07), pages 3176-3185, XP019883237, ISSN: 1573-4803, DOI: 10.1007/S10853-010-5201-1
- LAI ET AL.: 'Effect of Sc, Zr, and Ti on the interfacial reactions of the B,C/A1 systems'.' J MATER SCI vol. 46, no. 2, 2011, pages 451 - 459
- ZHANG ET AL.: 'Effect of titanium on microstructure and fluidity of A1-B4C composites'.' J MATER SCI vol. 46, no. 9, 2011, pages 3176 - 3185

## Description

This application claims priority from U.S. provisional patent application 61/727,949 filed on November 19, 2012.

### TECHNOLOGICAL FIELD

The present invention relates to cast aluminum/boron carbide composite metal matrix material having products obtained from a peritectic reaction to increase their fluidity prior to casting. The reaction products are obtained by using additives capable of undergoing a perictectic reaction with the boron of the boron carbide.

### BACKGROUND

"Effect of Sc, Zr, and Ti on the interfacial reactions of the B4C/AI system" - J. Lai, Z. Zhang, X.G. Chen, J Mater Sci, 46:451-459, 2011 relates to B₄C plates immersed in liquid aluminum alloyed with Sc, Zr and Ti to investigate the interfacial reaction between B₄C and liquid aluminum at 730°C.

US2003175543 discloses a hybrid composite reinforced metal matrix in which the metal is aluminum, aluminum alloy, or a magnesium alloy containing a relatively high percentage of aluminum. In addition to the reinforcement, which is typically alumina, the metal matrix also includes a hardening agent which is at least one intermetallic compound of aluminum with at least one second metal chosen from iron, nickel, titanium, zirconium, cobalt and niobium. CA2491429 discloses a cast article from an aluminum alloy having the following composition in weight percent: Silicon 6.0 - 25.0, Copper 5.0 - 8.0, Iron 0.05 - 1.2, Magnesium 0.5 - 1.5, Nickel 0.05 - 0.9, Manganese 0.05 -1.2, Titanium 0.05 - 1.2, Zirconium 0.05- 1.2, Vanadium 0.05 - 1.2, Zinc 0.05 - 0.9, Strontium 0.001 - 0.1, Phosphorus 0.001 - 0.1, and the balance is Aluminum, wherein the silicon-to-magnesium ratio is 10 - 25, and the copper-to-magnesium ratio is 4 - 15. US2009263277 discloses a L12 aluminum alloy having magnesium or nickel; at least one of scandium, erbium, thulium, ytterbium, and lutetium; at least one of gadolinium, yttrium, zirconium, titanium, hafnium, and niobium; and at least one ceramic reinforcement. Aluminum oxide, silicon carbide, aluminum nitride, titanium boride, titanium diboride and titanium carbide are suitable ceramic reinforcement particles.

To increase the fluidity of the molten Al-B₄C mixture, and as described in U.S. patent Serial No. 7,562,962, titanium can be added. When titanium is added to the mixture of molten aluminum metal and B₄C powder, reaction products are formed near the interface of the B₄C particles and the aluminum matrix which "poison" the B₄C particles. The reaction products are taught to shield the B₄C particles from the aluminum.

It would be highly desirable to be provided with means and methods of maintaining a proper fluidity of a molten Al-B₄C mixture prior to casting and shaping. The means and methods would preferably provide/maintain a fluidity amenable to shaping and/or casting in industrial settings.

### BRIEF SUMMARY

The present disclosure provides a method of preparing a cast composite material comprising aluminum, products of a peritectic reaction between an additive and boron as well as dispersed boron carbide particles. The presence of the products of the peritectic reaction maintains the fluidity of the molten composite material, prior to casting, and facilitate castability and shaping of the composite material.

In a first aspect not covered by the claims, the present disclosure provides a cast composite material comprising (i) aluminum, (ii) products of a peritectic reaction between an additive and boron, (iii) dispersed boron carbide particles and (iv) optionally titanium. The additive is selected from the group consisting of chromium, molybdenum, vanadium, niobium, zirconium, strontium, scandium, and any combination thereof. A sample of the composite material has a fluidity, after having been heated, prior to casting, to a temperature of about 700°C for about 120 minutes, corresponding to a cast length of at least 100 mm when measured using a mold having a groove for containing the sample, the groove having a width of about 33 mm, a height of between about 6.5 mm and about 4.0 mm and being downwardly inclined, from an horizontal axis, of about 10°. In an embodiment, the cast length of the sample is at least 190 mm.In another embodiment, the cast composite material is submitted to holding during a holding time and to casting during a casting time and wherein the holding time and the casting time amounts to 120 minutes. In another embodiment, the products of the peritectic reaction are provided by combining a molten aluminum or a molten aluminum alloy with the additive capable of undergoing the peritectic reaction (prior to the incorporation of boron carbide particles). In yet a further embodiment, the additive is selected from the group consisting of zirconium, strontium, scandium and any combination thereof. In another embodiment, the additive is scandium. In a further embodiment, the additive is strontium. In yet a further embodiment, the additive is zirconium. In an embodiment, the concentration (v/v) of the dispersed boron carbide particles is between 4% and 40% with respect to the total volume of the cast composite material. In such embodiment, the concentration (w/w) of the additive can be between 0.47% and 8.00% with respect to the total weight of the cast composite material and optionally, the composite material can further comprise titanium at a concentration (w/w) between 0.50% and 4.00% with respect to the total weight of the cast composite material. In another embodiment, the concentration (v/v) of the dispersed boron carbide particles is between 4.5% and 18.9% with respect to the total volume of the cast composite material. In such embodiment, the concentration (w/w) of the additive can be between 0.38% and 4.00% with respect to the total weight of the cast composite material and, optionally, the cast composite material further comprises titanium at a concentration (w/w) between 0.40% and 2.00% with respect to the total weight of the cast composite material. In another embodiment, the concentration (v/v) of the dispersed boron carbide particles is between 19.0% and 28.0% with respect to the total volume of the cast composite material. In such embodiment, the concentration (w/w) of the additive can be between 1.68% and 6.00% with respect to the total weight of the cast composite material and, optionally, the cast composite material can further comprise titanium at a concentration (w/w) between 1.80% and 3.00% with respect to the total weight of the cast composite material. In still another embodiment, the concentration (v/v) of the dispersed boron carbide particles is between 25.0% and 28.0% or between 28.0% and 33.0% with respect to the total volume of the cast composite material. In such embodiment, the concentration (w/w) of the additive can be between 0.94% and 4.00% with respect to the total weight of the cast composite material and, optionally, the cast composite material can further comprise titanium at a concentration (w/w) between 1.00% and 2.00% with respect to the total weight of the cast composite material.

According to a second aspect, the present disclosure provides a method of preparing a cast composite material. The method comprises: (a) combining (i) a molten aluminum alloy comprising an additive capable of undergoing a peritectic reaction with boron (ii) between 4 and 40 v/v % of a source of boron carbide particles based on a total volume of the cast composite material so as to provide a molten composite material comprising products of the peritectic reaction between the additive and boron and dispersed boron carbide particles provided the molten aluminum alloy is free of titanium, wherein: the additive is selected from the group consisting of chromium, molybdenum, vanadium, niobium, zirconium, strontium, scandium, and any combination thereof, the concentration of the additive being between 1.10% w/w and 8.00% w/w% with respect to the total weight of the cast composite material; a sample of the composite material has a fluidity, after having been heated, prior to casting, to a temperature of 700° C for 120 minutes, corresponding to a cast length of at least 100 mm when measured using a mold having a groove for containing the sample, the groove having a width of 33 mm, a height of between 6.5 mm and 4.0 mm and being downwardly inclined, from an horizontal axis, of 10°; and(b) casting the molten composite during a casting time so as to form the cast composite material, wherein the casting time is at least 20 minutes.

In an embodiment, the cast length is at least 190 mm. In still another embodiment, the method further comprises, prior to step (b), holding the molten composite material during a holding time and casting the molten composite during a casting time, wherein the holding time and the casting time amounts to 120 minutes. In still another embodiment, the method further comprises, prior to step (a), providing the molten aluminum alloy by combining a molten aluminum or a molten aluminum alloy with the additive capable of undergoing the peritectic reaction.

According to a third aspect not covered by the claims, the present disclosure provides a method of improving the casting and/or shaping properties of a molten composite material comprising aluminum, products of a peritectic reaction between an additive and boron, and dispersed boron carbide particles. Broadly, the method comprises combining (i) a molten aluminum alloy comprising the additive capable of undergoing a peritectic reaction with boron with (ii) a source of boron carbide particles so as to provide a molten composite material. The additive is selected from the group consisting of chromium, molybdenum, vanadium, niobium, zirconium, strontium, scandium, and any combination thereof. A sample of the composite material has a fluidity, after having been heated, prior to casting, to a temperature of about 700°C for about 120 minutes, corresponding to a cast length of at least 100 mm when measured using a mold having a groove for containing the sample, the groove having a width of about 33 mm, a height of between about 6.5 mm and about 4.0 mm and being downwardly inclined, from an horizontal axis, of about 10°.

According to a fourth aspect not covered by the claims, the present disclosure provides a method of facilitating shaping of a molten composite material of a molten composite material comprising aluminum, products of a peritectic reaction between an additive and boron, and dispersed boron carbide particles. Broadly, the method comprises combining (i) a molten aluminum alloy comprising the additive capable of undergoing a peritectic reaction with boron with (ii) a source of boron carbide particles so as to provide a molten composite material. The additive is selected from the group consisting of chromium, molybdenum, vanadium, niobium, zirconium, strontium, scandium, and any combination thereof. A sample of the composite material having a fluidity, after having been heated, prior to casting, to a temperature of about 700°C for about 120 minutes, corresponding to a cast length of at least 100 mm when measured using a mold having a groove for containing the sample, the groove having a width of about 33 mm, a height of between about 6.5 mm and about 4.0 mm and being downwardly inclined, from an horizontal axis, of about 10°.

### BRIEF DESCRIPTION OF THE DRAWINGS

Having thus generally described the nature of the invention, reference will now be made to the accompanying drawing in which:
**Figure 1** shows the loss of fluidity of molten aluminum mixture containing different lots of B₄C powder. Results are shown as fluidity (as measured as a cast length (in mm) of sample measured using a K-mold) in function of holding time in the furnace (in min) for various lots (A to E) of B₄C powders (30% v/v) added to molten aluminum at an initial temperature of 735°C. Results are shown for lot A containing 3.5% w/w Ti ( ), lot B containing 3.5% w/w Ti ( ), lot C containing 3.5% w/w Ti (A), lot D containing 3.0% w/w Ti (●) and lot E containing 2.0 % Ti w/w (○).
**Figure 2** illustrates an embodiment of a K-mold that can be used for determining the cast length of the composite material. (**A**) Schematic side elevation view of the lower inclined portion 10 of the K-mold. (**B**) Schematic top elevation view of the groove-containing portion 40 of the K-mold. (**C**) Schematic cross-sectional view of the groove-containing portion 40 of the K-mold.

### DETAILED DESCRIPTION

The fabrication of boron metal matrix composites (MMC) with high B₄C content (e.g., for example at least 30% v/v) usually requires B₄C powder of exceptional quality. High quality B₄C powders have a good granulometric distribution and have a minimum of fine powder-like particles. Generally, only such B₄C powder may be incorporated in high amounts into the metal matrix. When the B₄C powder is not of such good quality, significant losses of fluidity during the holding time of the molten metal, i.e. prior to casting, can be observed. In addition, increasing the holding temperature of the molten metal does not compensate for this loss of fluidity because this can favor the reaction between the aluminum and the B₄C powder thereby further increasing the viscosity (loss of fluidity). In such circumstances, the molten metal behaves as a thixotropic material.

Figure 1 shows the loss of fluidity during the holding time of a molten composite, prior to casting. In industrial settings, a certain fluidity is required for a certain amount of time for allowing the shaping/casting of the Al-B₄C mixture. The curves shown in Figure 1 show that the B₄C powder used in the preparation of the composite material increased the viscosity of the material and failed to meet the fluidity required in industrial settings for subsequent steps (shaping for example), even in the presence of titanium.

In accordance with the present disclosure, there is provided a cast Al-B₄C composite material comprising aluminum, products of a peritectic reaction and dispersed boron carbide particles. The composite material is obtained by first combining aluminum (or an aluminum alloy) with an additive (or a combination of additives) capable of undergoing a peritectic reaction with the boron of the boron carbide particles and ultimately provide products of such peritectic reaction in the aluminum or the aluminum alloy. Once the additive has been included in the aluminum (or in the aluminum alloy), boron carbide particles are combined with the aluminum (or the aluminum alloy), thereby causing the peritectic reaction between the additive and the boron. As shown herein, the use of the additive in the aluminum/aluminum alloy (and, ultimately the presence of peritectic reaction products in the composite material) has been shown useful for maintaining the fluidity of the molten composite and as such imparts good castability to a molten composite material. In some embodiments, it is believed that the use of the additive inhibits or slows down the formation of reaction products occurring during holding of the molten composite (such as, for example, the reaction products occurring between Al and B₄C). In other embodiments, it has been shown that the additives can be used to limit the use of titanium in such composite materials without altering substantially their fluidity. This maintenance in fluidity of the molten composite material can allow for the lengthening of the holding time of the molten mixture in the furnace, for using a lower grade of B₄C source as well as for facilitating shaping and/or casting of the resulting metal matrix composite(s).

Prior to being casted, the composite material is in a molten state and has a fluidity. In the disclosure described herein, the molten composite material has, prior to casting, a fluidity which permits casting in an industrial setting. In other to determine the fluidity of a molten composite material, it is possible to use a K-mold. Such mold, currently used and known in the art, measures the length of a sample of the composite material before it solidifies. The length measured with a K-mold is referred to as a cast length.

An embodiment of a K-mold that can be used to determine the fluidity of a sample of a molten composite material is shown in Figure 2. A K-mold is usually composed of two engageable portions, a lower inclined portion 10 (as shown in Figure 2A) and a groove-containing portion 40 (as shown in Figures 2B and 2C). When the sample is inserted in the mold, the inclined portion 10 is engaged with the groove-containing portion 40. The sample is allowed to cast along the inclined portion 10 and within the groove 50 until it sets. The length covered by the sample, usually measured in millimeters, is a measure of fluidity and refers to a cast length.

As shown on Figure 2A, the lower inclined portion is usually monolithic and comprises a plane 15 having a smooth surface and being downwardly inclined from an horizontal axis 20 by an angle 30 of about 10°. The plane 15 is for contacting directly the external sides 55 of the groove-containing portion 40 (shown on Figures 2B and 2C) and for providing an angle to the groove of about 10°.

The groove-containing portion 40 is a partially hollowed structure defining an enclosable groove 50 for containing the sample of the molten composite (Figure 2B). As shown on Figure 2B, the groove-containing portion has external sides 55 for contacting directly the plane 15 of the inclined portion 10. In the embodiment shown in Figure 2B, the groove 50 contains two different sections: sections 60 and sections 70 (defining a protuberance). In some embodiments, the K-mold comprises at least four sections 70 (e.g., four protuberances) located at a distance of 93 mm, 130 mm, 168 mm and 205 mm from the start of the mold (e.g., the position at which the sample starts contacting the inclined plane 15).

Figure 2C shows an enlarged of the enclosable groove 50. The sections 60 have a similar height 61 of about 6.5 mm. The height 61 is constant between the length defined by the external walls 55. The height 61 is measured with respect to the axis 80 defined by the inclined plane 15 (when the groove-containing portion 40 is engaged with the inclined portion 10). The sections 70 also have a similar height 71 of about 4 mm. The height 71 is constant between the length defined by the external walls 55. The height is measured with respect to the axis 80 defined by the inclined plane 15 (when the groove-containing portion 40 is engaged on the inclined portion 10).

In the context of the present disclosure, the cast composite material has a fluidity, preferably prior to casting, corresponding to a cast sample length of at least 100 mm, at least 120 mm, at least 140 mm, at least 160 mm, at least 180 mm, at least 190 mm or at least 200 mm. The sample used for determining the fluidity of the composite material can be heated at a temperature of about 700°C and for about 120 min to reproduce the industrial casting settings. Thus, the present disclosure also provides a method of manufacturing a cast composite material. In order to do so, a molten aluminum alloy (also referred to as an aluminum-base matrix alloy) comprising the additive (or a combination of additives) capable of undergoing the peritectic reaction is combined with a source of boron carbide to provide a molten composite. As shown in the present disclosure, the fluidity of the molten composite can be maintained at acceptable industrial levels for a longer period of time when compared to a similar molten composite which lacks the additive.

In the methods described herein, the aluminum or the aluminum alloy used is provided in a molten form. As such, the aluminum or the aluminum alloy is preferably heated to its melting temperature prior to its combination with the B₄C particles. In an embodiment, the aluminum alloy comprises (in embodiments consists essentially of and, in further embodiments, consists of) an additive capable of undergoing the peritectic reaction, the remainder being essentially aluminum or an aluminum alloy. Unavoidable or inevitable impurities (at the most 0.05 % w/w for each impurity) can also be present in the alloy (for a total of impurities of at most 0.15% w/w). Exemplary aluminum alloys include, but are not limited to, alloys from the 11xx series and from the 6xxx series. In some aspects not covered by the scope of the claims, Ti can be included in the aluminum or the aluminum alloy. In an alternative embodiment, if Ti is present in the aluminum or the molten aluminum alloy, it is considered to be a trace element (e.g. its concentration does not exceed the concentration of inevitable impurities).

In an embodiment, the composite material comprises between 4% and 40% (v/v) of B₄C particles and the molarity of the additive (or the combination of additives) in the composite material is between 0.01044 and 0.08351. In some aspects not covered by the scope of the claims, when Ti is present in the composite material, the combined molarity of the additive (or the combination of additives) and Ti is between 0.01044 and 0.08351. In some embodiments, the concentration of the additive in the composite material can be between 0.47% to 15.32%, 0.47% to 8.00%, 0.90% to 8.00%, 0.95% to 8.00%, 1.00% to 8.00% or 1.10% to 8.00% with respect to the total weight of the composite material (comprising the B₄C particles). In some aspects not covered by the claims, the combined concentration of the additive and Ti in the composite can be between 0.47% to 15.32%, 0.47% to 8.00%, 0.90% to 8.00%, 0.95% to 8.00%, 1.00% to 8.00% or 1.10% to 8.00% with respect to the total weight of the composite material (comprising the B₄C particles).

In another embodiment, the composite material comprises between 4.5% and 18.9% (v/v) of B₄C particles and the molarity of the additive (or the combination of additives) in the composite material is between 0.00835 and 0.04175. In some aspects not covered by the claims, when Ti is present in the composite material, the combined molarity of the additive (or the combination of additives) and Ti is between 0.00835 and 0.04175. In some embodiments, the concentration of the additive in the composite material can be between 0.38% to 7.68%, 0.38% to 4.00%, 0.90% to 4.00%, 0.95% to 4.00%, 1.00% to 4.00% or 1.10% to 4.00% with respect to the total weight of the composite material (comprising the B₄C particles). In some aspects not covered by the claims, the combined concentration of the additive and Ti in the composite can be between 0.38% to 7.68%, 0.38% to 4.00%, 0.90% to 4.00%, 0.90% to 4.00%, 1.00% to 4.00% or 1.10% to 4.00% with respect to the total weight of the composite material (comprising the B₄C particles).

In a further embodiment, the composite material comprises between 19% and 28% (v/v) of B₄C particles and the molarity of the additive (or the combination of additives) in the composite material is between 0.03758 and 0.06263. In some aspects not covered by the claims, when Ti is present in the composite material, the combined molarity of the additive (or the combination of additives) and Ti is between 0.03758 and 0.06263. In some embodiments, the concentration of the additive in the composite material can be between 1.69% to 11.51% or 1.69% to 6.00% with respect to the total weight of the composite material (comprising the B₄C particles). In some aspects not covered by the claims, the combined concentration of the additive and Ti in the composite can be between 1.69% to 11.51% or 1.69% to 6.00% with respect to the total weight of the composite material (comprising the B₄C particles).

In a further embodiment, the composite material comprises between 25% and 28% (v/v) or between 28% and 33% (v/v) of B₄C particles and the molarity of the additive (or the combination of additives) in the composite material is between 0.02088 and 0.04175. In some aspects not covered by the claims, when Ti is present in the composite material, the combined molarity of the additive (or the combination of additives) and Ti is between 0.02088 and 0.04175. In some embodiments, the concentration of the additive in the composite material can be between 0.94% to 7.68%, 0.94% to 4.00%, 0.95% to 4.00%, 1.00% to 4.00% or 1.10% to 4.00% with respect to the total weight of the composite material (comprising the B₄C particles). In some aspects not covered by the claims, the combined concentration of the additive and Ti in the composite can be between 0.94% to 7.68%, 0.94% to 4.00%, 0.95% to 4.00%, 1.00% to 4.00% or 1.10% to 4.00% with respect to the total weight of the composite material (comprising the B₄C particles).

The concentration of the additive, provided at a weight percent concentration or at a certain molarity, whether with reference to the aluminum alloy or the total composite material, is to be understood to include all forms of the additives (including soluble additive, excess additive that comes out of solution as intermetallics or refractory compounds, as well additive included in a B-containing peritectic reaction product). The additive capable of causing the formation of a peritectic reaction's product can be added in any convenient form, including master alloy (for example an AI-10% additive master alloy) or as additive-containing granules or powders. In some embodiments, it can be contemplated to add the additive as a form of a powder to wrought alloys (including AA1xxx, AA2xxx, AA3xxx, AA4xxx or AA6xxx) or casting alloys (including AA2xx or AA3xx).

Similarly, the titanium concentration or molarity given in the foregoing description, whether with reference to the aluminum alloy or the total composite material, represent titanium in all forms (including soluble Ti, excess Ti coming out of solution as intermetallics or refractory compounds, as well Ti-B compounds). In some aspects not covered by the claims, the titanium can be added in any convenient form, including master alloy (for example an AI-10% Ti master alloy) or as titanium containing granules or powders. In some aspects not covered by the claims, it may be advisable to use an AA1xxx alloy containing titanium in the aluminum alloy. In some aspects not covered by the claims, it can be contemplated to add a titanium as an aluminum alloy such as, for example, wrought alloys (including AA2xxx, AA3xxx, AA4xxx or AA6xxx), or casting alloys (including AA2xx or AA3xx).

In some embodiments, the additive capable of causing the formation of a peritectic reaction's product can be zirconium and the aluminum alloy can comprises or contains zirconium. In some embodiments, when Zr is used as an additive, the composite material does not comprise Ti (if present, Ti is considered to be a trace element). In some aspects not covered by the claims, when Zr is used as an additive, Ti can be present in the composite material. In a composite material comprising between 4% and 40% (v/v) of B₄C particles, zirconium can be provided at a concentration of between about 0.95 to about 7.61, between about 1.00 to about 7.61 or between about 1.10 to about 7.61 weight percentage with respect to the composite material's (comprising the B₄C particles) total weight. In such aspects not covered by the claims, when Ti is present, it can be provided at a concentration of between about 0.50 to about 4.00, between about 0.90 to about 4.00, between about 0.95 to about 4.00, between about 1.00 to about 4.00 or between about 1.10 to about 4.00 weight percentage with respect to the composite material's (comprising the B₄C particles) total weight. In a composite material comprising between 4.5% and 18.9% (v/v) of B₄C particles, zirconium can be provided at a concentration of between about 0.76 to about 3.81, between about 0.90 to about 3.81, between about 0.95 to about 3.81, between about 1.00 to about 3.81 or between about 1.10 to about 3.81 weight percentage with respect to the composite material's (comprising the B₄C particles) total weight. In such aspects not covered by the claims, when Ti is present, it can be provided at a concentration of between about 0.40 to about 2.00, between about 0.90 to about 2.00, between about 0.95 to about 2.00, between about 1.00 to about 2.00 or between about 1.10 to about 2.00 weight percentage with respect to the composite material's (comprising the B₄C particles) total weigh. In a composite material comprising between 19% and 28% (v/v) of B₄C particles, zirconium can be provided at a concentration of between about 3.43 to about 5.71 weight percentage with respect to the composite material's (comprising the B₄C particles) total weight. In some aspects not covered by the claims, when Ti is present, it can be provided at a concentration of between about 1.80 to about 3.00 weight percentage with respect of the composite material's (comprising the B₄C particles) total weight. In a composite material comprising between 25% and 28% (v/v) or 28% and 33% of B₄C particles, zirconium can be provided at a concentration of between about 1.90 to about 3.81 weight percentage with respect to the composite material's (comprising the B₄C particles) total weight. In some aspects not covered by the claims, when Ti is present, it can be provided at whereas titanium can be provided at a concentration between about 1.00 to about 2.00 or between about 1.10 to about 2.00 weight percentage with respect of the composite material's (comprising the B₄C particles) total weight. It will be understood that the zirconium concentrations given in the foregoing description, whether with reference to the aluminum alloy or the total composite material, represent zirconium in all forms (including soluble Zr, excess Zr coming out of solution as intermetallics or refractory compounds, as well Zr-B compounds). The zirconium can be added in any convenient form, including master alloy (for example an AI-10% Zr master alloy) or as zirconium containing granules or powders. In some embodiments, it may be advisable to use an AA1xxx alloy containing zirconium in the aluminum alloy. In alternative or complementary embodiments, it can be contemplated to add a zirconium as an aluminum alloy such as, for example, wrought alloys (including AA2xxx, AA3xxx, AA4xxx or AA6xxx), or casting alloys (including AA2xx or AA3xx).

In some embodiments, the additive capable of causing the formation of a peritectic reaction's product can be strontium and, in some aspects not covered by the claims, the aluminum alloy can comprises or contains strontium in combination with titanium. In a composite material comprising between 4% and 40% (v/v) of B₄C particles, strontium can be provided at a concentration of between about 0.91 to about 7.32, between about 0.95 to about 7.32, between about 1.00 to about 7.32 or between about 1.10 to about 7.32 weight percentage with respect to the composite material's (comprising the B₄C particles) total weight, whereas titanium can be provided at a concentration of between about 0.50 to about 4.00, between about 0.90 to about 4.00, between about 0.95 to about 4.00, between about 1.00 to about 4.00 or between about 1.10 to about 4.00 weight percentage with respect to the composite material's (comprising the B₄C particles) total weight. In a composite material comprising between 4.5% and 18.9% (v/v) of B₄C particles, strontium can be provided at a concentration of between about 0.73 to about 3.66, between about 0.90 to about 3.66, between about 0.95 to about 3.66, between about 1.00 to about 3.66 or between about 1.10 to about 3.66 weight percentage with respect to the composite material's (comprising the B₄C particles) total weight, whereas in some aspects not covered by the claims, titanium can be provided at a concentration of between about 0.40 to about 2.00, between about 0.90 to about 2.00, between about 0.95 to about 2.00, between about 1.00 to about 2.00 or between about 1.10 to about 2.00 weight percentage with respect to the composite material's (comprising the B₄C particles) total weight. In a composite material comprising between 19% and 28% (v/v) of B₄C particles, strontium can be provided at a concentration of between about 3.29 to about 5.49 weight percentage with respect to the composite material (comprising the B₄C particles) total weight, whereas in some aspects not covered by the claims, titanium can be provided at a concentration between about 1.80 to about 3.00 weight percentage with respect of the composite material's (comprising the B₄C particles) total weight. In a composite material comprising between 25% and 28% (v/v) or between 28% and 33% of B₄C particles, strontium can be provided at a concentration of between about 1.83 to about 3.66 weight percentage with respect to the composite material (comprising the B₄C particles) total weight, whereas in some aspects not covered by the claims, titanium can be provided at a concentration between about 1.00 to about 2.00 or between about 1.10 to about 2.00 weight percentage with respect of the composite material's (comprising the B₄C particles) total weight. It will be understood that the strontium concentrations given in the foregoing description, whether with reference to the aluminum alloy or the total composite material, represent strontium in all forms (including soluble Sr, excess Sr coming out of solution as intermetallics or refractory compounds, as well Sr-B compounds). The strontium can be added in any convenient form, including master alloy (for example an Al-10% Sr master alloy) or as strontium containing granules or powders. In some embodiments, it may be advisable to use an AA1xxx alloy containing strontium in the aluminum alloy. In alternative or complementary embodiments, it can be contemplated to add a strontium as an aluminum alloy such as, for example, wrought alloys (including AA2xxx, AA3xxx, AA4xxx or AA6xxx), or casting alloys (including AA2xx or AA3xx).

In some embodiments, the additive capable of causing the formation of a peritectic reaction's product can be scandium and the aluminum alloy can comprises or contains scandium in combination with titanium. In a composite material comprising between 4% and 40% (v/v) of B₄C particles, scandium can be provided at a concentration of between about 0.47 to about 3.75, between about 0.90 to about 3.75, between about 1.00 to about 3.75 or between about 1.10 to about 3.75 weight percentage with respect to the composite material's (comprising the B₄C particles) total weight, whereas in some aspects not covered by the claims, titanium can be provided at a concentration between about 0.50 to about 4.00, between about 0.90 to about 4.00, between about 0.95 to about 4.00, between about 1.00 to about 4.00 or between about 1.10 to about 4.00 with respect to the composite material's (comprising the B₄C particles) total weight. In a composite material comprising between 4.5% and 18.9% (v/v) of B₄C particles, scandium can be provided at a concentration of between about 0.38 to about 1.88, between about 0.90 to about 1.88, between about 1.00 to about 1.88 or between about 1.10 to about 1.88 weight percentage with respect to the composite material's (comprising the B₄C particles) total weight, whereas in some aspects not covered by the claims, titanium can be provided at a concentration of between about 0.40 to about 2.00, between about 0.90 to about 2.00, between about 0.95 to about 2.00, between about 1.00 to about 2.00 or between about 1.10 to about 2.00 weight percentage with respect to the composite material's (comprising the B₄C particles) total weight. In a composite material comprising between 19% and 28% (v/v) of B₄C particles, scandium can be provided at a concentration of between about 1.69 to about 2.82 weight percentage with respect to the composite material (comprising the B₄C particles) total weight, whereas in some aspects not covered by the claims, titanium can be provided at a concentration between about 1.80 to about 3.00 weight percentage with respect of the composite material's (comprising the B₄C particles) total weight. In a composite material comprising between 25% and 28% (v/v) or 28% and 33% of B₄C particles, scandium can be provided at a concentration of between about 0.94 to about 1.88, between about 1.00 to about 1.88 or between about 1.10 to about 3.88 weight percentage with respect to the composite material (comprising the B₄C particles) total weight, whereas in some aspects not covered by the claims, titanium can be provided at a concentration between about 1.00 to about 2.00 or between about 1.10 to about 2.00 weight percentage with respect of the composite material's (comprising the B₄C particles) total weight. It will be understood that the scandium concentrations given in the foregoing description, whether with reference to the aluminum alloy or the total composite material, represent scandium in all forms (including soluble Sc, excess Sc coming out of solution as intermetallics or refractory compounds, as well Sc-B compounds). The scandium can be added in any convenient form, including master alloy (for example an AI-10% Sc master alloy) or as scandium containing granules or powders. In some embodiments, it may be advisable to use an AA1xxx alloy containing scandium in the aluminum alloy. In alternative or complementary embodiments, it can be contemplated to add a scandium as an aluminum alloy such as, for example, wrought alloys (including AA2xxx, AA3xxx, AA4xxx or AA6xxx), or casting alloys (including AA2xx or AA3xx).

Without wishing to be bound to theory, the additive can be used in the methods described herein to form reaction products with B having an enthalpy of formation which is more negative than the one associated to AlB₂. For example, in some aspects not covered by the claims, when vanadium is used in an aluminum alloy comprising titanium, it is believed, without being bound by theory, that this addition would force another reaction with titanium. The reaction product could be a compound such as (Ti,V)B₂. The formation of such reaction products would stop or reduce the reaction between the aluminum melt containing titanium and the B₄C particles. The present disclosure thus provides for the addition of additive capable of causing the formation of a peritectic reaction's products as inhibitors of the reaction between the aluminum melt and the B₄C particles to maintain the fluidity of the composite until the composite is shaped, preferably cast.

Theoretical calculations of the enthalpy of formation of reaction products expected to form after the addition of various elements were carried out using the software FactStage^{™} and are shown in Table 1.

**Table 1. Theoretical values of enthalpy of formation of various reaction products.**

| Element added | Peritectic reaction product with B₄C | Enthalpy of formation (kJ/mol) |
|---|---|---|
| | **AIB₂** | **-67** |
| Cr | CrB₂ | -94 |
| Mo | MoB₂ | -150 |
| V | VB₂ | -202 |
| Ta | TaB₂ | -222 |
| Nb | NbB₂ | -251 |
| Ti | TiB₂ | -280 |
| Hf | HfB₂ | -320 |
| Zr | ZrB₂ | -326 |
| W | W₂B₉ | -375 |

In an embodiment, the additive includes, but is not limited to chromium (Cr), molybdenum (Mo), vanadium (V), niobium (Nb), hafnium (Hf), zirconium (Zr), strontium (Sr), scandium (Sc), tantalum (Ta), tungsten (W) as well as any combination thereof. In another embodiment, the additive includes, but is not limited to (Mo), vanadium (V), niobium (Nb), hafnium (Hf), zirconium (Zr), strontium (Sr), scandium (Sc) as well as any combination thereof. In still another embodiment, the additive includes, but is not limited to zirconium (Zr), strontium (Sr), scandium (Sc) as well as any combination thereof. In yet a further embodiment, the additive comprises or consists of Cr. In yet another embodiment, the additive comprises or consists of Mo. In still a further embodiment, the additive comprises or consists of V. In yet another embodiment, the additive comprises or consists of Nb. In another embodiment, the additive comprises or consists of Ta. In yet another embodiment, the additive comprises or consists of W. In still a further embodiment, the additive comprises or consists of Hf. In another embodiment, the additive comprises or consists of Zr. In yet a further embodiment, the additive comprises or consists of Sr. In still a further embodiment, the additive comprises or consists of Sc. In one embodiment, the additive comprises or consists of a combination of Zr and Sc. In another embodiment, the additive comprises or consists of a combination of Zr and Sr. In yet another embodiment, the additive comprises or consists of a combination of Sr and Sc. In yet another embodiment, the additive comprises or consists of a combination of Zr, Sr and Sc.

To provide the molten aluminum alloy, the additive(s), and in some aspects not covered by the claims optionally titanium, is (are) added to molten aluminum or to a molten aluminum or a molten aluminum alloy. In some embodiments, it is contemplated to mix/stir the elements of the molten aluminum alloy to obtain a substantially homogenous molten aluminum alloy. In alternative or complementary embodiments, it is contemplated to apply heat to the molten aluminum alloy to obtain a substantially homogenous molten aluminum alloy.

In some aspects not covered by the claims, and as indicated above, an aluminum alloy containing titanium can be used. In such embodiment, it is not necessary to add the titanium and the additive (or a combination of additives) in a specific order to the aluminum or aluminum alloy. In an embodiment, the titanium is first added to the molten aluminum/alloy and then the additive(s) is (are) added. In an alternative embodiment, the additive(s) is (are) first added to the molten aluminum/alloy and then the titanium is added. In still another embodiment, the titanium and the additive(s) are added simultaneously to the molten aluminum/alloy.

Once the molten aluminum alloy is provided, it is combined with a source of boron carbide (a boron carbide powder (such as a free-flowing powder) for example) to provide a molten composite material comprising dispersed boron carbide particles. In the molten composite material, it is understood that the aluminum alloy (supplemented with the additive and optionally titanium) is in a molten form and that the boron carbide particles are in a solid form and are at least partially in association with the products of the peritectic reaction. In some embodiments, it may be advisable to add the source of boron carbide (e.g., the boron carbide powder) to the molten aluminum alloy described herein. In some embodiments, it is contemplated to mix/stir the elements of the molten composite material to obtain a substantially homogenous molten composite material having dispersed B₄C-containing particles. The term "dispersed" means that the B₄C-containing particles are distributed substantially uniformly throughout the material's matrix. In some embodiments, it is contemplated that the mixing/stirring be carried out in a manner that allows the appropriate wetting of the B₄C particles in the composite material.

The molten composite material, due to the presence of the products of the peritectic reaction products, has a fluidity amenable for casting in an industrial setting. Fluidity can be determined by various ways as known by those skilled in the art. In one example, fluidity is measured with a viscometer. In another example, fluidity is assessed by measuring the length of a cast sample in a mold. In order to do so, it is possible to add a quantity of B₄C powder inside a reactor (capacity of about 35 kg for example) that contains liquid aluminum-based mixture at a specific temperature (about 700°C for example) to which a vacuum is applied. Samples of the mixture of molten metal and B₄C powder can be obtained at a fixed interval (for example, every 20 minutes) using a step-mold and having a predetermined length. In some embodiments, a K-mold step-mold can be used. Fluidity is quantified as the distance achieved/covered by the resulting mixture before its solidification. In some embodiments, the K-mold can be a graphite-coated stainless steel step-mould having a sample-receiving chamber or groove having a width of 33 mm (and, in some embodiments, a maximal length of 315 mm) and being inclined at an angle of about 10°. For example, a molten composite material achieving a distance of 100 mm after 120 minutes of holding time in the K-mold described above is considered as having a fair fluidity for direct chilled casting. In another example, a molten composite material achieving a distance of 190 mm after 120 minutes of holding time in the K-mold described above is considered as having an excellent fluidity for direct chilled casting. In an embodiment, the fluidity of the composite material is 190 mm or more after 120 min. In yet further embodiments, the fluidity of the composite material is of 200 mm or more after 120 minutes. In an embodiment, the fluidity of the molten composite is at least 100 mm when measured at a temperature of about 700°C after a holding time of 120 min. In embodiment, the fluidity of the composite material is at least 105 mm, 110 mm, 115 mm, 120 mm, 125 mm, 130 mm, 135 mm, 140 mm, 145 mm, 150 mm, 155 mm, 160 mm, 165 mm, 170 mm, 175 mm, 180 mm, 181 mm, 182 mm, 183 mm, 184 mm, 185 mm, 186 mm, 187 mm, 188 mm, 189 mm, 190 mm, 191 mm, 192 mm, 193 mm, 194 mm, 195 mm, 196 mm, 197 mm, 198 mm, 199 mm or 200 mm when measured at a temperature of about 700°C after a holding time of 120 min. In some embodiments, it is expected that the fluidity of the molten composite can vary upon holding time and holding temperature. In other embodiments, the fluidity of the composite material is not measured upon the mixture of the aluminum alloy and the boron carbide particles, but after the peritectic reaction products have been formed or even molten composite material is held at a specific temperature (e.g., holding temperature) and for a specific amount of time (e.g., holding time).

In embodiments, it is contemplated to hold a sample of the composite material at a specific temperature for allowing the material to remain in a molten state. In specific embodiments, the composite material is held at a minimal holding temperature of equal to or higher than about 660°C, 670°C, 680°C, 690°C, 700°C, 710°C, 720°C, 730°C, 740°C, 750°C, 760°C, 770°C, 780°C, 790°C or 800°C. In specific embodiments, the composite material is held at a maximal holding temperature equal to or lower than about 800°C, 790°C, 780°C, 770°C, 760°C, 750°C, 740°C, 730°C, 720°C, 710°C, 700°C, 690°C, 680°C, 670°C or 660°C. In alternative embodiments, the composite material is held at a temperature ranging between the minimal holding temperature as defined above and the maximal holding temperature as defined above.

In some embodiments, it is contemplated to hold a sample of the composite material in a molten state for a specific holding time. In specific embodiments, the composite material is held for a minimal holding time of equal to or higher than about 20 min, 30 min, 40, min, 50 min, 60 min, 70 min, 80 min, 90 min, 100 min ,110 min, 120 min, 130 min, 140 min, 150 min, 160 min, 170 min, 180 min, 190 min or 200 min. In specific embodiments, the composite material is held for a maximal holding time equal to or lower than about 200 min, 190 min, 180 min, 170 min, 160 min, 150 min, 140 min, 130 min, 120 min, 110 min, 100 min, 90 min, 80 min, 70 min, 60 min, 50 min, 40 min 30 min or 20 min. In alternative embodiments, the specific holding time ranges between the minimal holding time as defined above and the maximal holding time as defined above.

In some embodiments, it is contemplated to cast the composite material during a specific casting time. In specific embodiments, the composite material is casted for a minimal casting time of equal to or higher than about 20 min, 30 min, 40, min, 50 min, 60 min, 70 min, 80 min, 90 min, 100 min ,110 min, 120 min, 130 min, 140 min, 150 min, 160 min, 170 min, 180 min, 190 min or 200 min. In specific embodiments, the composite material is casted for a maximal casting time equal to or lower than about 200 min, 190 min, 180 min, 170 min, 160 min, 150 min, 140 min, 130 min, 120 min, 110 min, 100 min, 90 min, 80 min, 70 min, 60 min, 50 min, 40 min 30 min or 20 min. In alternative embodiments, the specific casting time ranges between the minimal casting time as defined above and the maximal casting time as defined above.

The molten composite is amenable any form of casting (including DC casting of billets or slabs), casting of ingots for future remelting and casting as well as casting into shapes using any convenient form of shape casting. The cast composite can be further processed and is well adapted for further operations such as (a) remelting and casting a shape, (b) extrusion and (c) rolling or (d) forging.

The method described herein may be used for the preparation of any shaped aluminum boron carbide composite material, particularly those containing high levels of B₄C. Advantageously, in some embodiments, in the presence of additive, a lower-grade B₄C powder can be used without altering significantly the fluidity of the molten Al-Ti-B₄C composite.

The present invention will be more readily understood by referring to the following examples which are given to illustrate the invention rather than to limit its scope.

### EXAMPLE I

A primary aluminum metal alloy (AA1100) was melted in a reactor at a temperature of 765°C. Ti was added and then Sr was added. Thereafter, B₄C particles were injected into the melt. The final concentrations of Ti and Sr were both 1.65 wt%. The final concentration of the B₄C particles was 28 vol %.

The final mixture was held at a temperature of about 700°C and two fluidity samples were obtained at given intervals starting 5 minutes after obtaining the final mixture. The fluidity measurements are shown in Table 2.

**Table 2. Fluidity measurements resulting from Example I.**

| **Time (min)** | **Fluidity measurement #1 (mm)** | **Fluidity measurement #2 (mm)** |
|---|---|---|
| 5 | 161 | 170 |
| 20 | 179 | 172 |
| 47 | 185 | 194 |
| 65 | 199 | 193 |
| 80 | 186 | 180 |
| 100 | 180 | 186 |
| **120** | **205** | **191** |

The results shown in Table 2 indicate that after a holding time of 120 minutes, the fluidity is higher than 190 mm, thereby allowing industrial casting of the composite material.

### EXAMPLE II

A primary aluminum metal alloy (AA1100) was melted in a reactor at a temperature of 765°C. Zr was added. Thereafter, B₄C particles were injected into the melt. The final concentration of Zr was 3.8 wt%. The final concentration of the B₄C particles was 19 vol %.

The final mixture was held at a temperature of about 700°C and two fluidity samples were obtained at various intervals. Resulting fluidity measurements are shown in Table 3.

**Table 3. Fluidity measurements resulting from Example II.**

| **Time (min)** | **Fluidity measurement (mm)** |
|---|---|
| 10 | 260 |
| 20 | 280 |
| 40 | 295 |
| 60 | 306 |
| 80 | 291 |
| 100 | 200 |
| **120** | **210** |

The results shown in Table 3 indicate that after a holding time of 120 minutes, the fluidity is still higher 190 mm, thereby allowing industrial casting of the composite material.

**Table 2. Fluidity measurements resulting from Example I.**

| **Time (min)** | **Fluidity measurement #1 (mm)** | **Fluidity measurement #2 (mm)** |
|---|---|---|
| 5 | 161 | 170 |
| 20 | 179 | 172 |
| 47 | 185 | 194 |
| 65 | 199 | 193 |
| 80 | 186 | 180 |
| 100 | 180 | 186 |
| **120** | **205** | **191** |

The results shown in Table 2 indicate that after a holding time of 120 minutes, the fluidity is higher than 190 mm, thereby allowing industrial casting of the composite material.

### EXAMPLE II

A primary aluminum metal alloy (AA1100) was melted in a reactor at a temperature of 765°C. Zr was added. Thereafter, B₄C particles were injected into the melt. The final concentration of Zr was 3.8 wt%. The final concentration of the B₄C particles was 19 vol %.

The final mixture was held at a temperature of about 700°C and two fluidity samples were obtained at various intervals. Resulting fluidity measurements are shown in Table 3.

**Table 3. Fluidity measurements resulting from Example II.**

| **Time (min)** | **Fluidity measurement (mm)** |
|---|---|
| 10 | 260 |
| 20 | 280 |
| 40 | 295 |
| 60 | 306 |
| 80 | 291 |
| 100 | 200 |
| **120** | **210** |

The results shown in Table 3 indicate that after a holding time of 120 minutes, the fluidity is higher 190 mm, thereby allowing industrial casting of the composite material.

While the invention has been described in connection with specific embodiments thereof, it will be understood that the scope of the claims should not be limited by the preferred embodiments set forth in the examples, but should be given the broadest interpretation consistent with the description as a whole.

## Claims

1. A method of preparing a cast composite material, said method comprising:
(a) combining (i) a molten aluminum alloy comprising an additive capable of undergoing a peritectic reaction with boron (ii) between 4 and 40 v/v % of a source of boron carbide particles based on a total volume of the cast composite material so as to provide a molten composite material comprising products of the peritectic reaction between the additive and boron and dispersed boron carbide particles provided the molten aluminum alloy is free of titanium, wherein:
• the additive is selected from the group consisting of chromium, molybdenum, vanadium, niobium, zirconium, strontium, scandium, and any combination thereof, the concentration of the additive being between 1.10% w/w and 8.00% w/w% with respect to the total weight of the cast composite material;
• a sample of the composite material has a fluidity, after having been heated, prior to casting, to a temperature of 700°C for 120 minutes, corresponding to a cast length of at least 100 mm when measured using a mold having a groove for containing the sample, the groove having a width of 33 mm, a height of between 6.5 mm and 4.0 mm and being downwardly inclined, from an horizontal axis, of 10°; and
(b) casting the molten composite during a casting time so as to form the cast composite material, wherein the casting time is at least 20 minutes.

2. The method of claim 1, wherein the alloy is an AA1XXX alloy.

3. The method of claim 1 or 2, further comprising, prior to step (a), providing the molten aluminum alloy by combining a molten aluminum or a molten aluminum alloy with the additive.

4. The method of any one of claims 1 to 3, wherein the additive is selected from the group consisting of zirconium, strontium, scandium and any combination thereof.

5. The method of claim 4, wherein the additive is zirconium, the concentration of the additive being between 1.10% w/w% and 7.61% w/w% with respect to the total weight of the cast composite material.

6. The method of claim 4, wherein the additive is strontium, the concentration of the additive being between 1.10% w/w% and 7.32% w/w% with respect to the total weight of the cast composite material.

7. The method of claim 4, wherein the additive is scandium, the concentration of the additive being between 1.10% w/w% and 3.75% w/w% with respect to the total weight of the cast composite material.

8. The method of anyone of claims 1 to 7, wherein the casting time is equal to or lower than 200 minutes.

9. The method of any one of claims 1 to 8, wherein the cast length is at least 105 mm.

## Patentansprüche

1. Verfahren zur Herstellung eines Gussverbundwerkstoffs, wobei das Verfahren umfasst:
(a) Kombinieren (i) einer geschmolzenen Aluminiumlegierung, die ein Additiv umfasst, das in der Lage ist, eine peritektische Reaktion mit Bor einzugehen, (ii) zwischen 4 und 40 Vol.-% einer Borcarbidteilchen-Quelle, bezogen auf ein Gesamtvolumen des Gussverbundwerkstoffs, um einen geschmolzenen Verbundwerkstoff bereitzustellen, der Produkte der peritektischen Reaktion zwischen dem Additiv und Bor, und dispergierte Borcarbidteilchen umfasst, vorausgesetzt, dass die geschmolzene Aluminiumlegierung frei von Titan ist, wobei:
- das Additiv ausgewählt ist aus der Gruppe bestehend aus Chrom, Molybdän, Vanadium, Niob, Zirconium, Strontium, Scandium, und einer Kombination davon, wobei die Konzentration des Additivs zwischen 1,10 Gew.-% und 8,00 % Gew.-%, bezogen auf das Gesamtgewicht des Gussverbundwerkstoffs, liegt;
- eine Probe des Verbundwerkstoffs, nachdem sie vor dem Gießen 120 Minuten lang auf eine Temperatur von 700 °C erhitzt wurde, eine Fließfähigkeit aufweist, die, unter Verwendung einer Form gemessen, welche eine Rille zum Aufnehmen der Probe aufweist, einer Gusslänge von mindestens 100 mm entspricht, wobei die Rille eine Breite von 33 mm, eine Höhe von zwischen 6,5 mm und 4,0 mm aufweist und von einer horizontalen Achse um 10° nach unten geneigt ist; und
(b) Gießen des geschmolzenen Verbunds während einer Gießzeit, um das Gussverbundmaterial zu bilden, wobei die Gießzeit mindestens 20 Minuten beträgt.

2. Verfahren nach Anspruch 1, wobei es sich bei der Legierung um eine AA1XXX-Legierung handelt.

3. Verfahren nach Anspruch 1 oder 2, das vor Schritt (a) weiter das Bereitstellen der geschmolzenen Aluminiumlegierung durch Kombinieren eines geschmolzenen Aluminiums oder einer geschmolzenen Aluminiumlegierung mit dem Additiv umfasst.

4. Verfahren nach einem der Ansprüche 1 bis 3, wobei das Additiv ausgewählt ist aus der Gruppe bestehend aus Zirconium, Strontium, Scandium, und einer Kombination davon.

5. Verfahren nach Anspruch 4, wobei es sich bei dem Additiv um Zirconium handelt, wobei die Konzentration des Additivs zwischen 1,10 % Gew.-% und 7,61 % Gew.-%, bezogen auf das Gesamtgewicht des Gussverbundwerkstoffs, liegt.

6. Verfahren nach Anspruch 4, wobei es sich bei dem Additiv um Strontium handelt, wobei die Konzentration des Additivs zwischen 1,10 % Gew.-% und 7,32 % Gew.-%, bezogen auf das Gesamtgewicht des Gussverbundwerkstoffs, liegt.

7. Verfahren nach Anspruch 4, wobei es sich bei dem Additiv um Scandium handelt, wobei die Konzentration des Additivs zwischen 1,10 % Gew.-% und 3,75 % Gew.-%, bezogen auf das Gesamtgewicht des Gussverbundwerkstoffs, liegt.

8. Verfahren nach einem der Ansprüche 1 bis 7, wobei die Gießzeit gleich oder kleiner als 200 Minuten ist.

9. Verfahren nach einem der Ansprüche 1 bis 8, wobei die Gusslänge mindestens 105 mm beträgt.

## Revendications

1. Procédé de préparation d'un matériau composite coulé, ledit procédé comprenant:
(a) combiner (i) un alliage d'aluminium fondu comprenant un additif capable de subir une réaction péritectique avec du bore (ii) entre 4 et 40% v/v d'une source de particules de carbure de bore par rapport au volume total du matériau composite coulé de manière à fournir un matériau composite fondu comprenant des produits de la réaction péritectique entre l'additif et le bore et des particules de carbure de bore dispersées à condition que l'alliage d'aluminium fondu soit exempt de titane, dans lequel :
• l'additif est choisi dans le groupe constitué par le chrome, le molybdène, le vanadium, le niobium, le zirconium, le strontium, le scandium et toute combinaison de ceux-ci, la concentration de l'additif étant comprise entre 1,10% p/p et 8,00% p/p% par rapport au poids total du matériau composite coulé ;
• un échantillon du matériau composite a une fluidité, après avoir été chauffé, avant la coulée, à une température de 700°C pendant 120 minutes, correspondant à une longueur coulée d'au moins 100 mm lorsqu'elle est mesurée en utilisant un moule ayant une rainure pour contenir l'échantillon, la rainure ayant une largeur de 33 mm, une hauteur comprise entre 6,5 mm et 4,0 mm et étant inclinée vers le bas, à partir d'un axe horizontal, de 10° ; et
(b) couler le composite fondu pendant une durée de coulée de manière à former le matériau composite coulé, où la durée de coulée est d'au moins 20 minutes.

2. Procédé de la revendication 1, dans lequel l'alliage est un alliage AA1XXX.

3. Procédé de la revendication 1 ou 2, comprenant en outre, avant l'étape (a), fournir de l'alliage d'aluminium fondu en combinant un aluminium fondu ou un alliage d'aluminium fondu avec l'additif.

4. Procédé de l'une quelconque des revendications 1 à 3, dans lequel l'additif est choisi dans le groupe constitué par le zirconium, le strontium, le scandium et toute combinaison de ceux-ci.

5. Procédé de la revendication 4, dans lequel l'additif est du zirconium, la concentration de l'additif étant comprise entre 1,10% p/p% et 7,61% p/p% par rapport au poids total du matériau composite coulé.

6. Procédé de la revendication 4, dans lequel l'additif est le strontium, la concentration de l'additif étant comprise entre 1,10% p/p% et 7,32% p/p% par rapport au poids total du matériau composite coulé.

7. Procédé de la revendication 4, dans lequel l'additif est du scandium, la concentration de l'additif étant comprise entre 1,10% p/p% et 3,75% p/p% par rapport au poids total du matériau composite coulé.

8. Procédé de l'une quelconque des revendications 1 à 7, dans lequel la durée de coulée est inférieure ou égale à 200 minutes.

9. Procédé de l'une quelconque des revendications 1 à 8, dans lequel la longueur coulée est d'au moins 105 mm.
